

## 1

2,990,296

## CHEMICAL PLATING OF METAL-BORON ALLOYS

Ralph M. Hoke, Fair Oaks, Calif., assignor to Callery Chemical Company, Pittsburgh, Pa., a corporation of Pennsylvania  
 No Drawing. Filed Aug. 5, 1958, Ser. No. 753,192  
 8 Claims. (Cl. 117—130)

This invention relates to a method of chemical plating and more particularly to a method of plating metal objects with metal-boron alloys.

Nickel-boron and cobalt-boron alloys are known for their superior flowing properties, wear resistance, and hardness. Metal boron alloys, or metal borides, are particularly useful as coatings for steel and other metals that do not possess these desirable properties. The metal-boron alloys are also useful as catalysts for a number of chemical reactions, e.g., hydrogenation reactions. Coatings of metal-boron alloys on other metallic base materials are particularly desirable as catalysts since a maximum amount of catalytic surface is provided by a minimum amount of the metal-boron alloy.

This invention is based on my discovery that an aqueous solution of an amine borane,  $X \cdot BH_3$  where X is an amine, and a soluble nickel or cobalt salt is a stable chemical plating solution. When a material with a catalytically active surface is contacted with this plating solution, a reaction occurs at the surface forming an adherent continuous plate of metal-boron alloy on the surface. The alloy plate itself is catalytically active so that the surface reaction can be continued to form a plate of any desired thickness. I have found that any clean metal surface, free of oxide film, is catalytically active. Glass, waxes, e.g. paraffinic waxes, natural fibers, and synthetic organic polymers, e.g. polyethylene and nylon, exhibit essentially no catalytic activity.

The solution or plating bath of this invention comprises an aqueous solution containing from about: (1) 0.02 to 6 parts by weight metal ion of the metal boron alloy to be plated, and (2) 0.1 to 3 parts by weight of borane radical,  $BH_3$ .

The metal ion, i.e. cobalt, or nickel ion, is provided by use of any soluble metal salt such as nickel sulfate, nickel chloride, nickel acetate, cobaltous sulfate, cobaltous chloride or other suitable soluble salts.

The borane radical is provided by the use of any secondary or tertiary amine borane, e.g. trimethylamine borane, dimethylamine borane, tripropylamine borane, pyridine borane and lutidine borane. Primary amine boranes are not satisfactory for use in the plating baths because they are rapidly decomposed by hydrolysis reactions.

The pH of the plating baths should be maintained below about 6.5; at higher pH values the plating reaction is extremely slow and some metal ion precipitates as the hydroxide. It is preferred to maintain the pH above about 2 because at lower pH values the solution is only metastable and tends to react spontaneously forming a large amount of particulate precipitate so that only a small proportion of the metal-boron alloy is plated. The initial pH of the aqueous plating solutions containing the metal salt and the amine borane are within the preferred range. As the plating reaction proceeds the pH of the solution increases because of the release of amine from the reacted amine borane. If the pH increases to too high a value, the solution can be acidified with any non-oxidizing acid, e.g. HCl. It is particularly convenient to buffer the plating solution with a weak, non-oxidizing acid, e.g. acetic acid or boric acid.

The plating baths of this invention have varying degrees of activity; the more active baths plate at a higher rate. The activity of the bath increases with increasing metal

## 2

ion concentration and increasing borane radical concentration. The activity of the bath also increases with a decrease in pH. The plating bath may be used at any temperature between about room temperature and the boiling point of the solution with the activity of the bath increasing with increasing temperature.

The object to be plated is immersed in the plating bath and the plating commences. The object may conveniently be suspended by a string or rope made of natural or synthetic fiber, or it may be suspended in a cloth or supported by a wood, glass, or synthetic polymer rack. If a metal piece is used to support the object to be plated, some of the bath will be consumed in plating the support. After the object has been plated, it is removed from the bath and washed with water to remove the bath solution and permitted to dry.

Metal objects to be plated must have clean surfaces free of oxide film. The objects are cleaned by any of the conventional cleaning procedures. The clean metal surface catalyzes the chemical reduction reaction which results in a metal-boron alloy plate on the clean surface. Objects of steel, iron, nickel, cobalt, titanium, copper and copper base alloys, aluminum and aluminum base alloys, palladium, and other metals may be plated according to this invention.

It is preferred to contain the plating solution in a vessel that exposes only non-active surfaces to the bath. Glass vessels are most convenient, and synthetic polymer vessels, such as polyethylene vessels, and vessels lined with non-active material may be used, e.g., paraffin wax lined, polyethylene lined, or polyvinylidene chloride lined vessels. The plating process is then selective; the plating occurs on the metal object immersed in the solution and does not occur on the vessel walls.

When plating has proceeded for several hours, a small amount of metal-boron alloy particulate precipitate is formed and collects at the bottom of the vessel. This precipitate is itself catalytically active so that if it is not removed some of the plating solution will be consumed by reaction induced by the precipitate. The precipitate may be removed by filtration.

The chemical plating consumes borane radical and metal ion; any desired concentration or concentration range may be maintained by adding additional amine borane or metal salts to the plating solution.

The following examples are illustrative of the plating solutions of this invention. The compositions of the solutions are expressed in weight percent of anhydrous reactants. The actual metal salts used were hydrates.

## Example I

A plating solution containing 0.95 wt. percent



5.14 wt. percent  $NiCl_2$ , and 93.91 wt. percent water was made by adding the amine borane to an aqueous solution of nickel chloride contained in a glass vessel. Clean metal strips of copper, Phosphor bronze, brass, antimonial Admiralty, Olympic bronze, cartridge brass, nickel, Inconel, Monel, cupro nickel, aluminum, and carbon steel were plated with nickel-boron alloy by immersing the individual metal strips in aliquots of the plating solution for two hours at about 25° C.

## Example II

65 A plating solution was prepared which contained 0.95 wt. percent  $(CH_3)_2NH \cdot BH_3$ , 5.14 wt. percent  $NiCl_2$ , and 93.91 wt. percent water. The pH of the solution was 5.4. A carbon steel test panel was immersed in the solution maintained at 18° C. for 2 1/3 hours. A nickel-boron alloy immediately started to plate on the steel panel. During the course of the plating reaction the pH increased to 6.13

and the rate of plating decreased. The average rate of plate-deposition was  $0.019 \times 10^{-3}$  inches per hour.

*Example III*

The rate of formation of boron alloy plate is increased if the solution is buffered to reduce the increase in pH during the course of the reaction. For example, a buffered solution containing 3.7 wt. percent  $(\text{CH}_3)_2\text{NH}\cdot\text{BH}_3$ , 9.3 wt. percent  $\text{NiCl}_2$ , 2.5 wt. percent  $\text{H}_3\text{BO}_3$  and 84.5 wt. percent water had a pH of 4.25. A nickel-boron alloy was plated on a carbon steel panel immersed in the solution for 6½ hours at 18° C. The average plating rate was  $0.091 \times 10^{-3}$  inches per hour.

*Example IV*

An adherent continuous nickel-boron plate was formed at an average rate of  $0.014 \times 10^{-3}$  inches per hour on a carbon steel panel by immersing it in a plating solution at 24° C. for 127 minutes. The plating solution contained 1.1 wt. percent  $(\text{CH}_3)_3\text{N}\cdot\text{BH}_3$ , 5.1 wt. percent  $\text{NiCl}_2$ , and 93.8% water.

*Example V*

A carbon steel test panel was immersed in a plating solution containing 2.2 wt. percent  $(\text{CH}_3)_2\text{NH}\cdot\text{BH}_3$ , 5.1 wt. percent  $\text{CoCl}_2$ , and 92.7 wt. percent water. The average plating rate was  $0.03 \times 10^{-3}$  inches per hour for a two hour immersion at room temperature. During the plating reaction a small amount of particulate boron alloy precipitate was formed.

*Example VI*

A buffered plating solution containing 3.7 wt. percent  $(\text{CH}_3)_2\text{NH}\cdot\text{BH}_3$ , 10.1 wt. percent  $\text{CoCl}_2$ , 2.5 wt. percent  $\text{H}_3\text{BO}_3$ , and 83.7 wt. percent water had a pH of 4.02. A carbon steel panel was immersed in the solution at room temperature for 297 minutes. A bright plate of cobalt-boron alloy was plated on the panel at an average rate of  $0.25 \times 10^{-3}$  inches per hour.

The nickel-boron coatings formed by the process of this invention generally appear dark to semi-bright and the cobalt-boron coatings generally appear semi-bright to bright. The plated alloys contain from about 4 to 10 percent boron.

According to the provisions of the patent statutes, I have explained the principle and mode of practicing my invention, and have described what I now consider to be its best embodiments. However, I desire to have it understood that within the scope of the appended claims,

the invention may be practiced otherwise than as specifically described.

I claim:

- 5 1. An aqueous chemical plating solution containing as essential components (1) a compound selected from the group consisting of secondary and tertiary amine boranes and, (2) a compound selected from the group consisting of soluble salts of nickel and cobalt, the proportions of each component being such that the concentration of borane radical is between about 0.1 to 3 wt. percent, and the concentration of metal ion is between about 0.02 and 6 wt. percent.
- 10 2. A method of plating metal-boron alloys on metal objects which comprises the step of contacting the object to be plated with an aqueous plating solution containing as essential components (1) a compound selected from the group consisting of secondary and tertiary amine boranes and, (2) a compound selected from the group consisting of soluble salts of nickel and cobalt, the proportions of each component being such that the concentration of borane radical is between about 0.1 to 3 wt. percent and the concentration of metal ion is between about 0.02 and 6 wt. percent.
- 15 3. A method according to claim 2 in which the amine borane is dimethylamine borane.
- 20 4. A method according to claim 2 in which the pH of the plating solution is maintained between about 2 and 6.5.
- 25 5. A method according to claim 4 in which the pH is maintained by buffering the solution with a weak non-oxidizing acid.
- 30 6. A method according to claim 5 in which the acid is boric acid.
- 35 7. A method according to claim 2 in which the borane radical concentration is maintained by the periodic addition of amine borane.
- 40 8. A method according to claim 2 in which the metal ion concentration is maintained by the periodic addition of a soluble metal salt.

**References Cited in the file of this patent**

**UNITED STATES PATENTS**

- |           |                          |               |
|-----------|--------------------------|---------------|
| 2,461,661 | Schlesinger et al. ----- | Feb. 15, 1949 |
| 2,726,170 | Warf -----               | Dec. 6, 1955  |

**OTHER REFERENCES**

- Hurd: "Chemistry of the Hydrides," 1952 John Wiley and Sons, pg. 84.

**Notice of Adverse Decision in Interference**

In Interference No. 98,469 involving Patent No. 2,990,296, R. M. Hoke,  
Chemical plating of metal-boron alloys, final judgment adverse to the patentee  
was rendered Nov. 24, 1964, as to claims 1, 2, 3, 4, 5, 7 and 8.  
[*Official Gazette January 19, 1965.*]